

J. J. MANNING & J. W. STEPHENSON.  
MALLEABLE IRON CASTING AND METHOD OF MAKING SAME.  
APPLICATION FILED NOV. 28, 1904.

922,791.

Patented May 25, 1909.

Fig. 1.



Fig. 2.



WITNESSES

Thomas W. Bascom  
Lindell A. Pomeroy

INVENTORS

John J. Manning  
John W. Stephenson

# UNITED STATES PATENT OFFICE.

JOHN J. MANNING AND JOHN W. STEPHENSON, OF TOLEDO, OHIO, ASSIGNEES TO THE NATIONAL MALLEABLE CASTINGS COMPANY, OF CLEVELAND, OHIO, A CORPORATION OF OHIO.

## MALLEABLE-IRON CASTING AND METHOD OF MAKING SAME.

No. 922,791.

Specification of Letters Patent.

Patented May 25, 1909.

Application filed November 28, 1904. Serial No. 234,498.

To all whom it may concern:

Be it known that we, JOHN J. MANNING and JOHN W. STEPHENSON, both of Toledo, Lucas county, Ohio, have invented a new and useful Malleable-Iron Casting and Method of Making the Same, of which the following is a full, clear, and exact description, reference being had to the accompanying drawings, forming part of this specification, in 10 which—

Figure 1 is a side elevation partly in section of a journal-box embodying our invention; and Fig. 2 is a plan view partly in horizontal section.

der the box objectionable by reason of multiplying the parts. The composition which we prefer to use for the inserted cast iron piece is cast iron containing more manganese than is contained in cast iron from which malleable boxes are made. We can make such composition conveniently by adding to the ordinary mixture which is employed for making the cast malleable boxes sufficient manganese to make the total manganese in the iron from 2 to 4 per cent., and we cast the resistance piece from material of this composition, which we find is not substantially altered by the annealing process. A greater percentage of manganese may be employed.

In the drawings, 2 represents a journal-box of malleable cast iron having lateral guiding grooves 3, 3 for the pedestals of the truck. In casting the box we place in the mold inserts in the nature of channel-shape pieces 4, 4 which have been previously cast of the manganese composition above mentioned, and then cast the material of the box around them. We also may insert a similar piece 5 at the top of the box to constitute a bearing surface for the equalizer of the truck. We may make these inserted pieces continuous channels adapted to extend from end to end of the groove with lateral projections *b*, *b* by which they are confined to the box when the latter is cast around them; or as shown at 4', we may make these pieces so that they will extend only partially along the groove, and we may form in them conical-shape holes *c*, *c* in which the metal of the box will embed itself forming keys by which the pieces are held in place. Those skilled in the art will be able to devise other ways of shaping the pieces and casting them to the box. Within the scope of our invention as broadly claimed it may be applied to the facing of coupler knuckles and other articles of malleable cast iron so as to give them hard wearing surfaces, since

What we claim is:

1. An annealed malleable casting having included therein an insert having a manganese content to render the same capable of resisting annealing, substantially as described.
2. The herein described method which consists in including in a cast an insert having a manganese content to render the

15 A serious objection has been found in the use of journal boxes made of malleable cast iron when applied to pedestal trucks, in that the softness of the malleable iron causes it to wear rapidly, and in a relatively short time 20 the box must be taken out and scrapped. Facing material of steel or like hard metal applied to the box for the purpose of preventing this wear is unsatisfactory because if it be applied in a separate piece it complicates the manufacture and makes the box unduly expensive, and if it be attempted to apply it by uniting it to the box in the operation of casting, it is objectionable because the subsequent annealing operation which 25 is required to convert the material of the box from ordinary gray iron to malleable cast iron will destroy the temper of the inserted steel piece and will thus render it comparatively useless. We have discovered means 30 by which these difficulties can be overcome, and the journal-box provided with a durable wearing face which will enable it to outlast the ordinary malleable box and does not entail any objectionable features in the way of 35 expense or difficulty of manufacture.

To this end our invention consists in inserting in the box during the operation of casting at the places where the wear is to be resisted, a piece of cast iron of such composition that 40 it will resist the annealing process and will not be converted thereby into malleable iron.

The annealing process therefore converts only the main body of the box into malleable iron giving to it the desired qualities of 45 strength and toughness, while the inserted piece of cast iron retains its original properties of hardness and resistance to wear, and being an integral part of the box it does not substantially increase the expense, nor ren-

same capable of resisting annealing, and then annealing the casting with the insert therein, substantially as described.

3. An annealed malleable casting having a wear plate insert included therein during the casting operation and having a manganese content to render the same capable of resisting annealing, substantially as described.

4. The herein described method which 10 consists in placing in a mold an insert having a manganese content to render the same

capable of resisting annealing, pouring the mold; and thereafter annealing the casting with the insert therein, substantially as described.

In testimony whereof, we have hereunto set our hands, November 22, 1904.

JOHN J. MANNING.

JOHN W. STEPHENSON.

Witnesses:

THOMAS W. BAKEWELL,  
H. M. CORWIN.